

## UNITED STATES PATENT OFFICE

2,497,536

## YARN CONDITIONING

Carroll F. Chandler, Waynesboro, Va., assignor to  
E. I. du Pont de Nemours & Company, Wil-  
mington, Del., a corporation of Delaware

No Drawing. Application June 14, 1946,  
Serial No. 676,849

2 Claims. (Cl. 117—139.5)

1

This invention relates to the dressing of textile fibers, filaments and yarns and more particularly to improved finish compositions for fibers, filaments and yarns of cellulose acetate and the like.

In preparation for subsequent operations such as spooling, throwing, dyeing, etc., and in some cases to improve the appearance and hand, it is customary to dress the freshly spun yarn with a finish composition which generally comprises one or a mixture of oils such as mineral oils, drying oils, animal oils, vegetable oils, sulfonated oils; antioxidants, wetting agents, anti-static agents, sizes and a variety of other materials, both organic and inorganic, commonly in aqueous solution, emulsion or dispersion. This treatment serves one or a number of the following purposes: to prevent abrasion or breakage of the yarn during twisting or spooling, to counteract or offset the effects of static charges (particularly in the case of cellulose acetate), to facilitate dyeing of the yarn package, to increase tensile strength, tenacity and weight of the yarn to some extent, to impart to the yarn luster, softness and/or flexibility, to bond the fibers or filaments of the yarn, etc. The exact composition employed depends, of course, on the effects desired, but it is most difficult to formulate a composition which is satisfactory in every respect and it is especially difficult to formulate a finish composition which will not adversely affect the package or cake formation of headless packages.

An object of this invention therefore is to provide improved compositions with which to dress textile fibers, filaments and yarns.

Another object is to provide aqueous finish emulsions which will produce substantial improvements in yarn frictional properties and yarn quality.

Still another object is to treat cellulose acetate yarn whereby to secure better package formation and yarn of improved quality. These and other objects will more clearly appear hereinafter.

Unexpectedly, I have found that the presence on yarn of a relatively small amount of polyvinyl alcohol, applied as a constituent of the usual aqueous oil emulsion type of dressing, works a remarkable improvement in the quality and handling characteristics of the yarns and, in particular, imparts to the yarn a lower coefficient of friction.

2

Briefly stated therefore, my invention comprises applying to freshly formed artificial yarn, derived from any source, from 0.005% to 0.075%, based on the dry weight of the treated yarn, of a polyvinyl alcohol contained in an aqueous oil emulsion finish composition.

The term "polyvinyl alcohol" appearing herein is used in its accepted trade sense and denotes the water-soluble types of partially saponified and fully saponified polyvinyl acetate. For purposes of the present invention, it is preferred to use polyvinyl alcohols of low viscosity, i. e., polyvinyl alcohols having a maximum solution viscosity of 5 to 10 centipoises in 4% aqueous solution at 25° C. The amount of polyvinyl alcohol incorporated in the yarn must be maintained within the limits of 0.005% to 0.075% by weight, based on the dry weight of the treated yarn. If more than 0.075% of polyvinyl alcohol is used, poor cake formation occurs, there is sticking to under layers (especially after aging), crocking on guides and, in general, the results are unsatisfactory. The use of polyvinyl alcohol in accordance with the principles of this invention is not to be confused with its use as a yarn size, for in the present case, the amount of polyvinyl alcohol is insufficient to give a sizing effect; i. e., there is no filament or thread-to-thread adhesion as in sized yarn. Moreover, the advantages of sizing are generally related only to dried yarn, whereas the advantages of this invention are realized more particularly with yarn that has not been submitted to a drying action.

As a finish or lubricant composition, there may be employed any of the usual aqueous emulsions containing mineral, vegetable and/or animal oil, sulfonated oils, amine salts, anti-static agents, polyhydric alcohols, etc. which have heretofore been used in the dressing of textile fibers, filaments and yarns. The concentration of polyvinyl alcohol in the dressing composition will depend, of course, upon the amount of composition applied to the yarn and should be adjusted to provide an amount of polyvinyl alcohol in the yarn within the limits hereinabove specified.

To more fully illustrate the practice and advantages of this invention, the following example is given. Parts and percentage composition are by weight unless otherwise indicated.

50

## Example I

75 denier, 50 filament, 3.0 turn cellulose acetate yarn of 54.5% combined acetic acid containing

3.4% (calculated as solids) of a finish of the following composition:

|                                                                                            | Per cent |    |
|--------------------------------------------------------------------------------------------|----------|----|
| Sulfonated peanut oil                                                                      | 21.5     | 5  |
| Diethylene glycol                                                                          | 2.2      |    |
| 45% potassium hydroxide                                                                    | 1.1      |    |
| White mineral oil (#50)                                                                    | 58.2     |    |
| Oleic acid                                                                                 | 10.2     |    |
| Triethanolamine                                                                            | 4.9      | 10 |
| 40% solution of a "Dowicide A" (Dow sodium salt of phenyl phenate)                         | 1.4      |    |
| Polyvinyl alcohol (86-89% saponified; saponification No. 127-157; viscosity—5 centipoises) | 0.5      | 15 |

(applied as a water emulsion containing 22.7% solids) was tube wound, without drying, into three pound packages. Compared with three pound packages of identical yarn wound in the same way and dressed with the same relative amount of a finish composition (regular finish) containing no polyvinyl alcohol but otherwise identical with that specified above, the following results were observed:

|                                   | Polyvinyl Alcohol Finish | Regular Finish |
|-----------------------------------|--------------------------|----------------|
| Coefficient of friction           | 0.54                     | 0.62           |
| Per cent Reject packages          | 4.9                      | 10-15          |
| Warp Defects/Million Thread Yds.: |                          |                |
| Major Defects                     | 110                      | 250            |
| Minor Defects                     | 435                      | 1350           |
| Total Defects                     | 535                      | 1600           |

In addition, the package formation was excellent, and there was no objectionable crocking on guide or roll surfaces.

#### Example II

75 denier, 50 filament, 3.0 turn cellulose acetate yarn of 54.5% combined acetic acid containing about 3.4% (calculated as solids) of a finish of the following composition:

|                                       | Percent |
|---------------------------------------|---------|
| Butyl acetyl ricinoleate              | 10.0    |
| Triethanolamine oleate                | 22.3    |
| Sulfonated peanut oil                 | 10.0    |
| White mineral oil (#43)               | 42.2    |
| Propylene glycol                      | 3.0     |
| White mineral oil (#105)              | 6.9     |
| Diethylcyclohexylamino lauryl sulfate | 4.5     |
| Stenol (cetyl and stearyl alcohols)   | 1.1     |

prepared as a 25% aqueous emulsion to which is added 0.75% (calculated on the dry weight of the total finish solids) of polyvinyl alcohol (86-89% saponified, saponification No. 127-157, viscosity—5 centipoises), was tube wound, as in the previous example, without drying, into three pound packages. Compared with three pound packages of identical yarn wound in the same way and dressed with the same amount of finish composition (regular finish) containing no polyvinyl alcohol but otherwise identical with that specified above, the following results were observed:

|                                   | Polyvinyl Alcohol Finish | Regular Finish |
|-----------------------------------|--------------------------|----------------|
| Coefficient of friction           | 0.54                     | 0.60           |
| Per cent Reject packages          | 6.4                      | 7.9            |
| Warp Defects/Million Thread Yds.: |                          |                |
| Major Defects                     | 144                      | 368            |
| Minor Defects                     | 614                      | 1428           |
| Total Defects                     | 758                      | 1796           |
| Knots/3 lb. Cone                  | 3.6                      | 3.7            |
| Per cent 1-knot Cones             | 19                       | 12.3           |

Although this invention has been specifically illustrated in connection with the tube winding of headless packages of cellulose acetate yarn, it will be obvious to those skilled in the textile yarn art that it is applicable with like effect to other operations such as skeining, throwing, etc., and may be applied with advantage to textile fibers, filaments, yarn or threads of any other material, such as regenerated cellulose from viscose, cuprammonium cellulose, cellulose ethers or other cellulose derivatives, vinyl polymers, nylon, poly acrylonitrile, mercerized cotton, etc.

It will be apparent from the foregoing that this invention not only enables the production of yarn of improved quality, but, in addition, by reason of fewer rejects, lessened gumming of guides, rolls, etc., it contributes materially to the economy of such production. Moreover, it has been observed that the presence of small amounts of polyvinyl alcohol serves, in general, to stabilize the finish composition and to improve roll coverage where roll applicators are employed.

As many widely different embodiments can be made without departing from the spirit and scope of this invention, it is to be understood that the invention is not restricted in any way except as defined in the appended claims.

I claim:

1. In the process of conditioning textile filaments of synthetic, organic, filament-forming material wherein the freshly formed filament is dressed with an oil-containing, aqueous finish composition, the improvement which comprises incorporating in said finish composition sufficient polyvinyl alcohol to deposit on the filament from 0.005% to 0.075% by weight, based on the weight of the filament, of polyvinyl alcohol.

2. In the process of conditioning cellulose acetate filaments wherein the freshly formed filament is dressed with an oil-containing, aqueous finish composition, the improvement which comprises incorporating in said finish composition sufficient polyvinyl alcohol to deposit on the filament from 0.005% to 0.075% by weight, based on the weight of the filament, of polyvinyl alcohol.

CARROLL F. CHANDLER.

#### REFERENCES CITED

60 The following references are of record in the file of this patent:

#### UNITED STATES PATENTS

| Number    | Name     | Date           |
|-----------|----------|----------------|
| 1,920,564 | Jochum   | Aug. 1, 1933   |
| 2,132,901 | Jochum   | Oct. 11, 1938  |
| 2,381,587 | Griffin  | Aug. 7, 1945   |
| 2,385,714 | La Piana | Sept. 25, 1945 |